

Patented Feb. 9, 1926.

1,572,458

# UNITED STATES PATENT OFFICE.

WILLIAM P. WOODSIDE AND CHARLES NEUMAN DAWE, OF DETROIT, MICHIGAN, AS  
SIGNORS TO THE STUDEBAKER CORPORATION, OF SOUTH BEND, INDIANA, A COR-  
PORATION OF NEW JERSEY.

## ALLOY STEEL.

No Drawing.

Application filed August 24, 1923. Serial No. 659,213.

*To all whom it may concern:*

Be it known that we, WILLIAM P. WOOD-  
SIDE and CHARLES NEUMAN DAWE, citizens of  
the United States of America, and residents  
5 of Detroit, in the county of Wayne and State  
of Michigan, have invented certain new and  
useful Improvements in Alloy Steel, of  
which the following is a specification.

This invention relates to an alloy steel,  
10 more particularly designed for use in the  
manufacture of articles requiring a tough  
elastic core, and a hard outer surface adapted  
to form a bearing or wearing surface, such  
15 as pins, bolts, gears, bearings and other ma-  
chine parts.

Such articles are usually made from what  
is known as low carbon steel, that is, steel  
or alloy steel having such a low carbon con-  
tent that heating and quenching does not  
20 harden it to a material degree, it being nec-  
essary to carburize the surface by well known  
methods and then to properly heat and  
quench the same to obtain the desired sur-  
face hardness; the core, not having been car-  
25 burized, remaining relatively soft.

Heretofore, the steels available for such use  
have been such that the desired uniform  
hardness of the surface could only be ob-  
tained by heating, after carbonization, to the  
30 proper degree, and then quenching in water  
instead of oil. The great and very impor-  
tant disadvantage of quenching such articles  
in water is that while the desired hardness  
may be obtained, the surface is very brittle,  
35 whereas it is desirable that the surface be  
hard and at the same time tough and rela-  
tively elastic. Such articles as pins and the  
like invariably warp in the operation of  
quenching, whether the quenching agent be  
40 water or oil, and it is necessary to straighten  
them before grinding the surface to finished  
dimensions. Such articles quenched in water  
are so brittle that a relatively large percent-  
age are broken in the straightening oper-  
45 ation, and further, a relatively large percent-  
age of those successfully straightened have  
to be scrapped due to checks developing in  
their surface during the subsequent grinding  
operation, due to the excessive brittleness of  
50 the surface. The surface of such articles  
quenched in oil are not brittle but are tough  
and elastic. The hardness obtained by  
quenching these articles, made from the here-  
tofore available steels or alloy steels, in oil,

has been so low that it is considered prefer- 55  
able to obtain the desired surface hardness  
by quenching in water at the expense of the  
relatively large resulting percentage of  
scrap.

The object of our present invention is to 60  
provide an alloy steel that may be used for  
the manufacture of such articles, and which  
after having been properly carburized,  
heated and quenched in oil will have a sur- 65  
face hardness comparable with such articles  
made of the steels heretofore available and  
quenched in water, which because of their  
toughness and elasticity, may be straightened  
70 or bent with little, if any, breakages, and  
which will not develop surface checks in the  
operation of grinding. Another object is to  
provide such an alloy steel that will be cap-  
able of production on a commercial scale 75  
and at a cost commensurate with the cost of  
steels heretofore used for such purposes, and  
which will be readily capable of being rolled,  
forged, machined and the like.

Our invention consists in a new alloy steel  
having substantially or approximately the 80  
usual carbon and manganese content of mild  
steel and in addition thereto and alloyed  
therewith nickel preferably in the propor-  
tion of about 1.40 per cent to about 1.75 per  
85 cent and molybdenum, preferably in the pro-  
portion of about .20 per cent to about .30 per  
cent of the entire metal. The metal of  
our invention may and ordinarily does con-  
tain the usual small percentages of sulphur 90  
and phosphorus found in mild or low carbon  
steels.

Analyses of specimens of our improved  
alloy steel have shown compositions within  
the following limits: Carbon, .10% to .23%;  
manganese, .30% to .60%; sulphur, .06%  
max.; phosphorus, .04% max.; nickel, 1.40% 95  
to 1.75%; molybdenum, .20% to .30%; iron,  
97.02% to 98.00%.

We prefer to maintain the composition as  
to the essential elements within the limits  
indicated above, but obviously a slight ex-  
cess or deficiency of any of the elements of  
the composition would not involve a substan-  
tial change in the character of the steel and  
would be within our invention.

In the following claims the reference to 100  
mild steel is to be understood as implying  
the presence of carbon and manganese in  
about the proportions in which they com-

monly occur in mild or low carbon steel, such as is commonly employed for the purpose referred to above.

This alloy steel may be readily rolled, forged, machined and the like, its characteristics during such operations being approximately the same as in nickel steels having the same nickel content. The strength is approximately the same as other alloy steels having the same heat treatment, which is in the neighborhood of 30% greater than ordinary steel of the same carbon content.

We have found that this alloy steel particularly lends itself to the manufacture of parts to be machined from hot rolled or cold drawn bars, such as shackle-bolts, tie-rod bolts, worms, piston-pins and the like. These parts do not require heat treatment before the carburizing operation, and when heated, after having been carburized, from 1475 to 1500 degrees Fahrenheit and quenched in oil, they have a uniform surface scleroscope hardness after grinding of 75 to 85. As before stated, no steel has been available heretofore for such uses as described, which would give this uniform surface hardness by quenching in oil. Not only is the surface of articles made from this alloy steel quenched in oil as hard as described above, but the surface, while being of such a hardness, is tough and elastic, cracks but very little due to bending or straightening and is not so susceptible to the development of surface checks in the operation of grinding as in alloy steels heretofore used. It is therefore a particularly desirable alloy steel for use in the manufacture of such articles.

Having thus described our invention, what we claim is:

40 1. An alloy metal composed of .10% to .23% of carbon, .30% to .60% of manganese,

1.40% to 1.75% of nickel, .20% to .30% of molybdenum and 97% to 98.1% of iron.

2. An alloy steel having .10% to .23% of carbon, .30% to .60% of manganese, 1.00%<sup>45</sup> to 2.00% of nickel, and .15% to .30% of molybdenum.

3. A mild steel containing as alloying metals in addition to manganese substantial amounts of nickel and molybdenum only,<sup>50</sup> each of these metals being present in substantial proportions and the entire content of alloying metals not exceeding 2.66 per cent.

4. A mild steel containing from about 1.40 per cent to about 1.75 per cent nickel and from about .20 per cent to about .30 per cent of molybdenum.

5. A mild steel containing a small but substantial fraction of 1 per cent of molybdenum and from about 1.40 per cent to about 1.75 per cent of nickel.

6. A mild steel containing about .20 per cent to about .30 per cent of molybdenum and a larger percentage of nickel, the entire content of alloying metal not substantially exceeding 2.66 per cent.

7. A mild steel containing substantial amounts of nickel and molybdenum, the nickel being in excess of the molybdenum and the entire content of alloy metals not being substantially in excess of 2.66 per cent.

8. A mild steel containing from about .20 per cent to about .30 per cent of molybdenum and a larger percentage of nickel, the entire amount of alloying metals not substantially exceeding 2.66 per cent.

Signed by us at Detroit, Michigan, U. S. A.  
this 20th day of August, 1923.

WILLIAM P. WOODSIDE.  
C. NEUMAN DAWE.